

Aug. 30, 1960

N. J. CULP

2,950,968

DEEP-HARDENED ALLOY STEEL HAVING IMPROVED IMPACT STRENGTH

Filed May 31, 1957

2 Sheets-Sheet 2

FIG. 2



RELATION OF IMPACT STRENGTH TO  
COPPER ADDITIONS AS A FUNCTION OF  
MANGANESE PLUS COPPER CONTENT

Aug. 30, 1960

N. J. CULP

2,950,968

DEEP-HARDENED ALLOY STEEL HAVING IMPROVED IMPACT STRENGTH

Filed May 31, 1957

2 Sheets-Sheet 2

FIG. 2



RELATION OF IMPACT STRENGTH TO  
COPPER ADDITIONS AS A FUNCTION OF  
MANGANESE PLUS COPPER CONTENT

1

2,950,968

DEEP-HARDED ALLOY STEEL HAVING  
IMPROVED IMPACT STRENGTH

Neil J. Culp, West Lawn, Pa., assignor to The Carpenter Steel Company, Reading, Pa., a corporation of New Jersey

Filed May 31, 1957, Ser. No. 662,805

8 Claims. (Cl. 75—125)

This invention relates to alloy steels capable of deep hardening in large sections and more particularly to an alloy steel which to an enhanced degree embodies the capability of being readily deep hardened in large sections and which has improved impact properties.

There has long been a demand for alloy steels which in addition to being capable of deep hardening in large sections are also tough at room temperature. Alloys hitherto in use as tool and die steels have been deficient in one or the other of these properties. Such alloys having desirable impact properties are not capable of being deep hardened. Those having desirable deep hardening properties have poor impact properties.

By deep hardenability I refer to steels which are capable of being oil or air hardened throughout in sections as large as four inches in diameter by four inches long or larger. It has been generally characteristic of alloy steels that with an increase of the alloy content to improve the hardenability capability there has been a decrease in their toughness. Furthermore, even at relatively low carbon levels, it has been necessary to temper tool and die steels before they attain their limited impact strength. The alloy set forth in U.S. Patent No. 2,355,224 is illustrative of a composition which has an outstanding degree of deep hardenability but has relatively poor impact strength.

As a practical matter, it is desirable for such steels to be susceptible to heat treatment at as low a temperature as possible from which they are cooled in oil or air to provide deep hardenability. Thus, if a steel can be deep hardened in large sections from hardening temperatures at or below 1650° F. their use is greatly facilitated. It is also desirable, for the purpose of facilitating use of the composition in the field as well as elsewhere, for such steels to have a broad austenitizing temperature range, i.e., the steel should deep harden upon cooling from any temperature within a rather broad range. This is particularly advantageous in that it is then not necessary to utilize equipment which is specially adapted to maintain the temperature of the work within a critical and narrow temperature range. Thus, if a steel can be deep hardened from only such a narrow austenitizing temperature range of 100° F. or less it is far more difficult for fabricators to produce uniform results in making their products than if the austenitizing temperature range is a band of 150° F. or 300° F. This is especially the case when the composition does not require tempering to attain its optimum toughness.

Toughness, as measured by the notched bar impact test, is a very desirable property in steels capable of deep hardening but it is characteristic thereof that such steels require tempering before achieving their optimum impact strength. It is an important feature of my invention that when my alloy has a carbon content of about 0.45% or less tempering is not required to bring it to optimum toughness. When the carbon content is increased and is above about 0.45% tempering may be re-

2

quired to avoid excessive brittleness due to the hardening treatment.

Another very desirable property of alloy steels of this character is that they have good toughness at low temperatures because of the many applications in which such steels are necessarily exposed to low temperatures. In the past, it has been considered practically essential to include a substantial amount of nickel if a hardened steel is not to lose what toughness it has at room temperature when the temperature is lowered. Another important feature of my invention is that when my alloy has a carbon content not greater than about 0.45% it has good sub-zero, —100° F. or lower, impact properties and is not subject to the well known transition temperature effect. This as well as other unique properties are achieved in my compositions without more than the residual amounts of nickel that are obtained as impurities in melting alloy steels. Such amounts are usually only a few hundredths of 1%, usually less than about 0.2%.

It is an object of this invention to provide an alloy steel which is capable of deep hardening from a broad austenitizing range of temperature; which is capable of deep hardening from temperatures below about 1650° F.; and which has good toughness, as indicated by the notched bar impact test, in the as-quenched or the as-quenched and tempered condition. Another object is to provide such an alloy steel which retains a considerable proportion of its toughness at temperatures down to —100° F. or even lower. I have found that in order to achieve the unique combination of all of these properties, it is necessary to prepare an alloy steel in which the following alloying elements are present within the rather narrow ranges as indicated:

|            | Percent  |
|------------|----------|
| Carbon     | 0.2-0.8  |
| Manganese  | 0.5-2.5  |
| Chromium   | 0.5-1.5  |
| Molybdenum | 0.25-1.5 |
| Copper     | 0.65-4   |

and in which the relative amounts of carbon, manganese and copper are carefully controlled. As will be more fully pointed out hereinafter, when manganese is present in an amount of only about 0.5% then minimum amounts of about 2% copper and about 0.45% carbon are required to provide an alloy having all of the foregoing properties. The remainder of my composition is substantially iron which is intended to include such impurities as is consistent with good commercial practice as well as such additional elements which may be in keeping with good metallurgical practice but do not impair the aforementioned desirable properties of my composition. For example, from the standpoint of good melting practice, I include various amounts of silicon up to about 1%, while such elements as phosphorus and sulphur are preferably present only in residual amounts. Though vanadium does not appear to have any effect on the impact properties or hardenability of my composition, I may include up to about 0.5% when its effect in providing grain refinement is desired.

In the accompanying drawings, Figures 1 and 2 are graphs showing relationships between the alloying elements, carbon, copper and manganese.

Alloys of this composition can be hardened throughout, in air or oil, in sections, four inches in diameter and four inches long or larger to a Rockwell C hardness of around 40 to 65, after heating to a temperature within a range of 1500° F. to 1650° F. when the carbon content ranges from about 0.5% to about 0.8% while with lower carbon content the treating temperature range is even broader, being from 1500° F. to 1800° F. Such alloys also exhibit excellent toughness, as indi-

cated by notched bar impact tests. With a carbon content of up to about 0.45% such excellent toughness is exhibited even in the as-quenched condition and, while these compositions, like other alloy steels, gradually become less tough as the temperature is lowered, from room temperature to sub-zero temperatures, they exhibit no sharp decrease in toughness as they are cooled to extremely low temperatures but retain a considerable proportion of their room temperature toughness even when used at the low temperatures that exist in arctic climates.

While my composition may deep-harden with as low a carbon content as 0.1% it should contain at least 0.2% carbon in order to provide a satisfactory as-hardened hardness bearing in mind that the attainable heat treated hardness decreases as carbon is reduced although the impact strength improves. Too much carbon detracts from the air-hardenability, probably due to the formation of alloy carbides. The upper limit for carbon, therefore, is about 0.8% although lower amounts of carbon are preferable for numerous uses to which the alloy may be put. Articles such as chisels, for example, should contain carbon in the lower portion of the range given, while articles such as hardened steel dies may be made from alloys containing carbon in the upper portion of the range.

Chromium is present primarily to provide oxidation resistance and to reduce scale formation during hot working which occurs heavily below about 0.5%. Too much chromium adversely affects the low temperature impact properties. For this reason it is not desirable to employ more than about 1.5% chromium. Molybdenum, as well as chromium, is normally considered useful as contributing to the hardenability of alloy steels. However, I have found that molybdenum does not contribute to hardenability to the degree which would be normally anticipated and mainly affects the impact properties of my alloy. For the purpose of obtaining enhanced impact properties I preferably use up to about 1% molybdenum although somewhat more, up to about 1.5%, may be tolerable with the lower carbon contents of up to about 0.4%. Below about 0.25%, molybdenum is not present in sufficient quantity to provide the desired effect while above about 1.5% molybdenum has an undesirable effect on the impact properties of my composition. When chromium and/or molybdenum are utilized in amounts effective to provide deep hardenability, above 1.5%, the hardening temperature as well as the impact properties are adversely affected to a marked degree.

Copper and manganese affect both the hardenability and the impact properties of my compositions. As will be more fully pointed out hereinafter the carbon content largely controls the amounts of copper and manganese required to provide the minimum deep hardenability in such large sections although for the lower chromium and molybdenum contents I may use somewhat more copper and manganese. The copper and manganese also affect the temperature from which the alloys of the present invention can be fully hardened in minimum sections of four inches in diameter by four inches long. The addition of copper makes it possible to maintain a low hardening temperature of 1650° F. maximum. However, at about 0.5% manganese at least about 2% copper is required to maintain the low hardening temperature while below those quantities the manganese and copper are not present in sufficient amounts to provide the desired relatively low hardening temperature. From Figure 1 it is apparent that with about 0.5% manganese, a minimum of about 2% copper is required to provide the minimum air hardenability required to attain Rockwell C-59 in a four inch diameter by four inch long section with a carbon content of about 0.6%. Manganese has a greater effect than copper on hardenability and at the lower carbon levels I utilize

closer to maximum amounts of manganese to attain the required hardenability. Where quenching in oil may be utilized the smaller amounts of manganese and copper are satisfactory.

5 The curve of Figure 1 is based upon data obtained from specimens of my composition having a carbon content of about 0.6% and with a chromium and molybdenum content each of about 1%. Compositions falling under the curve do not contain enough manganese and copper for sufficient air hardenability to attain a minimum hardness of Rockwell C-59 in a minimum four inch by four inch section. The specimens were formed from ingots which were processed by forging and rolling and were heated at a temperature of 1600° F. for about 10 minutes and then air quenched. The weight percent of manganese is plotted along the horizontal scale while the weight percent of copper is plotted along the vertical scale. The point on the curve corresponding to 2% manganese, nil copper identifies the composition hereinbefore referred to in connection with Patent No. 2,355,224 which has relatively poor impact properties.

I have found that a unique improvement in impact properties both at room temperature and at extremely low temperatures is obtained in accordance with my invention by carefully utilizing copper and manganese in amounts which depend upon the carbon content of the composition. The relationship between the three elements, carbon, copper and manganese, is such that in 25 my preferred composition, in addition to the criteria hereinabove set forth, the value of the ratio of the copper content to the combined copper and manganese content must be maintained between critical limits which must be raised as the carbon content is increased from 30 0.2%. In Figure 2, lines A and B are plotted to show the minimum and maximum values respectively of the value of this ratio defined as the percent by weight of copper of the total or combined percent by weight of the manganese and copper content of the composition. 35 The curves of Figure 2 are based on data obtained from tests conducted on specimens having the composition of the examples enumerated in Table I and also on specimens having compositions as shown in Table II. For these tests specimens  $\frac{1}{2}$  inch by  $\frac{1}{2}$  inch by 40 2 $\frac{1}{2}$  inches long were processed and tested in accordance with the standard established by the American Society for Testing Materials. As shown by such standard notched bar impact tests, alloys of my composition for which the percent of copper of the combined copper-manganese content falls between lines A, B in Figure 45 50 55 2 all show a minimum improvement in toughness of at least 50% as compared to deep hardenable alloy steels hitherto known to me. Further, below about 0.45% carbon my composition does not require tempering but demonstrates exceptional impact strength in its as-quenched condition.

At any carbon level, plotted along the vertical scale in 60 Figure 2, lines A, B define along the horizontal scale the values in percent of the ratio of the percent copper content to the combined percent content of manganese and copper to provide the improved impact properties of this invention but without regard to the aforementioned desirable hardenability or the low treating temperature. Thus with 0.30% carbon the copper content should form 65 at least 20% of the total manganese and copper content but no more than 62%. With 0.6% carbon the copper content should form at least 61%. At and above 0.6% carbon, manganese is not required to provide the improved impact properties and is included, at least about 0.5%, to provide a minimum as-hardened hardness of 70 Rockwell C-59, and the low treating temperature. When copper is present in amounts above about 4% such undesirable metallurgical phenomena as precipitation of copper are likely to occur when the alloy is hardened and drawn. As the manganese content is increased above 75

2.5% the composition becomes difficult to anneal commercially. To achieve a minimum hardness of Rockwell C-59 throughout with air quenching in a four inch round with 0.5% manganese and 0.6% carbon a minimum of 2% copper is required (Figure 1). In order to extend the hardenability to even larger sections at this carbon and hardness level I may include up to about 4% copper. As shown in Figure 2 such an alloy is characterized by the improved impact properties of my invention.

Table I

| Example No. | C   | Mn   | Cr   | Mo   | Cu   | Hardenability  |
|-------------|-----|------|------|------|------|----------------|
| 1           | .29 | 1.52 | .75  | .60  | 1.80 | Air Hardening. |
| 2           | .31 | 1.60 | .88  | .67  | 1.30 | Do.            |
| 3           | .31 | 1.92 | .81  | .61  | 1.25 | Do.            |
| 4           | .34 | 1.33 | .10  | .70  | 1.42 | Do.            |
| 5           | .39 | 1.04 | 1.06 | .62  | .68  | Oil Hardening. |
| 6           | .39 | .49  | .74  | .69  | .89  | Do.            |
| 7           | .41 | .92  | 1.02 | .30  | .68  | Do.            |
| 8           | .42 | .91  | 1.06 | .30  | 1.31 | Do.            |
| 9           | .41 | 1.59 | 1.07 | .30  | 1.25 | Air Hardening. |
| 10          | .47 | .55  | .85  | .67  | 1.33 | Do.            |
| 11          | .62 | .11  | 1.00 | 1.02 | 1.00 | Oil Hardening. |
| 12          | .61 | .11  | 1.00 | 1.02 | 1.98 | Do.            |
| 13          | .60 | .11  | 1.00 | 1.02 | 2.89 | Air Hardening. |
| 14          | .64 | .51  | 1.08 | 1.04 | 1.04 | Air Hardening. |
| 15          | .64 | .51  | 1.08 | 1.04 | 2.00 | Air Hardening. |
| 16          | .64 | .51  | 1.08 | 1.04 | 3.00 | Do.            |

The relative amounts of copper and manganese at the different carbon levels of Examples 1-16 all fall between lines A, B of Figure 2. The careful balance of the alloying elements required is demonstrated by the results from similar tests conducted on specimens having the composition of the examples enumerated in Table II, the specimens having been processed as was indicated in connection with Table I.

Table II

| Example No. | C   | Mn   | Cr   | Mo   | Cu   | Hardenability  |
|-------------|-----|------|------|------|------|----------------|
| 17          | .29 | 1.50 | .75  | .61  | 2.80 | Air Hardening. |
| 18          | .29 | 1.48 | .75  | .61  | 3.68 | Do.            |
| 19          | .39 | 1.04 | 1.06 | .63  | .15  | Oil Hardening. |
| 20          | .39 | 1.04 | 1.06 | .63  | .34  | Do.            |
| 21          | .51 | 1.72 | .78  | .88  | 1.54 | Air Hardening. |
| 22          | .60 | 1.72 | .78  | .85  | 1.54 | Do.            |
| 23          | .64 | 1.00 | 1.03 | 1.06 | 1.03 | Do.            |
| 24          | .64 | 1.00 | 1.03 | 1.06 | 1.50 | Do.            |
| 25          | .64 | 1.00 | 1.03 | 1.06 | 2.03 | Do.            |
| 26          | .65 | 1.48 | 1.03 | 1.02 | .30  | Do.            |
| 27          | .65 | 1.48 | 1.03 | 1.02 | 1.03 | Do.            |
| 28          | .65 | 1.48 | 1.03 | 1.02 | 1.49 | Do.            |
| 29          | .63 | 1.96 | 1.05 | 1.08 | .51  | Do.            |
| 30          | .62 | 1.96 | 1.05 | 1.08 | 1.06 | Do.            |
| 31          | .71 | 1.72 | .78  | .85  | 1.54 | Do.            |

Specimens having the composition of the examples of Table II do not show the unique improvement in toughness which is characteristic of those set forth in Table I and when plotted in Figure 2 fall outside of the area between lines A and B. However, those compositions containing 0.2% to 0.45% carbon and in which copper constitutes from about 20% to 80% of the combined manganese and copper content, are characterized by desirable and advantageously useful properties. This is also the case of those compositions having a carbon content of 0.45% to 0.8% and in which copper constitutes at least 40% of the combined manganese and copper content.

Specimens having the following base compositions were prepared for purposes of comparison.

Table III

| Alloy Type | C   | Mn   | Cr   | Mo   | Cu   | Hardenability  |
|------------|-----|------|------|------|------|----------------|
| D          | .32 | 2.72 | .82  | .63  | 1.22 | Air Hardening. |
| E          | .50 | 1.94 | .98  | 2.01 | Nil  | Do.            |
| F          | .64 | 1.96 | 1.05 | 1.08 | .10  | Do.            |

Alloy D proved to be unannealable while alloys E and F had relatively poor impact strength even when com-

pared to the compositions of Table II. Alloy F will be recognized as a base composition of the patent hereinabove referred to.

Alloys of my composition are readily hot workable. 5 No difficulty was encountered in casting melts into ingots and processing them by forging and rolling to round cornered square bars.

The effect of manganese and copper on the hardening temperature and/or hardenability is shown by the 10 hardness attained in a minimum section of four inches diameter by four inches long. The results are given in Table IV where for convenience the manganese and copper contents are also included:

Table IV

| Example No. | Mn   | Cr   | Hardening Temperature, 1,600° F., Rockwell C | Hardening Temperature, 1,650° F., Rockwell C |
|-------------|------|------|----------------------------------------------|----------------------------------------------|
| F           | 1.96 | .10  | 63                                           | 63                                           |
| 26          | 1.48 | .50  | 61/63                                        | 63                                           |
| 23          | 1.00 | 1.03 | 59                                           | 61                                           |
| 25          | 1.00 | 2.03 | 62                                           | 62                                           |
| 14          | .51  | 1.04 | 48/49                                        | 53/54                                        |
| 16          | .51  | 3.00 | 60                                           | 61                                           |
| 13          | .11  | 2.89 | 47/48                                        | 53                                           |
| 11          | .11  | 1.00 | 38/39                                        | 42                                           |

From Table IV it is apparent that as the manganese content is reduced and the copper content is increased, the 30 composition has the desired relatively low hardening temperature. When in any one of my alloys the manganese content is below about 0.50% and the copper content is below about 2% then the low hardening temperature is not maintained.

35 The effect of excessive chromium on the low temperature impact properties of my composition is apparent from a comparison of the test results obtained from specimens having the composition of Example 4 but containing 0.89% chromium with the results obtained

40 from a similar composition containing 2.18% chromium. Keyhole Charpy impact measurements were made on such specimens which had been air hardened from 1650° F. The specimens containing 0.89% chromium had a hardness of Rockwell C 51/52 and gave measurements of 19-24 ft.-lbs. at room temperature, 20-17 ft.-lbs. at

45 0° F., and 16-18 ft.-lbs. at -100° F. On the other hand, specimens with 2.18% chromium had a hardness of Rockwell C 48 and gave measurements of 19-15 ft.-lbs. at room temperature, 11-12 ft.-lbs. at 0° F., and 2-8 ft.-lbs. at -100° F. The sharp drop in impact strength at the higher chromium level illustrates the adverse effect of excessive amounts of this element on the toughness of the composition.

50 Table V shows the improvement in impact properties for impact pieces treated in the center of a six inch diameter by six inch long section from a temperature of 1600° F. and tempered at 350° F. for one hour.

Table V

| Example | Mn   | Cu   | Hardness RC | Guillory Notch Charpy Average of 3 tests, ft.-lbs. |
|---------|------|------|-------------|----------------------------------------------------|
| F       | 1.96 | .10  | 60          | 7.5                                                |
| 30      | 1.96 | 1.06 | 60          | 10.5                                               |
| 24      | 1.00 | 1.50 | 60          | 13.5                                               |
| 25      | 1.00 | 2.03 | 59.5        | 10.5                                               |
| 16      | .51  | 3.00 | 59.5        | 17.0                                               |

55 Izod impact tests on specimens of Example 10, containing .47% carbon, air hardened from 1650° F. but not tempered and having a hardness of Rockwell C-58 resulted in measurements of 17-21 ft.-lbs. Similarly treated 60 specimens containing 0.31 carbon, 1.54 manga-

nese, 0.82 chromium, 0.65 molybdenum and 1.30 copper resulted in measurements of 50-55 ft.-lbs. Tests conducted on specimens of the last mentioned composition are illustrative of the exceptional low temperature impact properties of my composition. The specimens were air hardened from 1650° F. and again were not tempered. In the following table the results in foot pounds are shown together with the testing temperature and the as-hardened hardness.

| Testing Temp. | Keyhole Charpy, ft.-lbs. | Hardness, Rockwell C |
|---------------|--------------------------|----------------------|
| Room          | 19-24                    | 49                   |
| 0° F.         | 20-17                    | 50                   |
| -50° F.       | 19-18                    | 49                   |
| -100° F.      | 16-18                    | 50                   |
| -300° F.      | 7-10                     | 50                   |

The absence of a transition temperature effect in my compositions having up to about 0.45% carbon makes them especially valuable for use in applications where low and extremely low temperature conditions may be encountered.

The terms and expressions which have been employed are used as terms of description and not of limitation, and there is no intention, in the use of such terms and expressions, of excluding any equivalents of the features shown and described or portions thereof, but it is recognized that various modifications are possible within the scope of the invention claimed.

I claim:

1. A hardened alloy steel article having good impact strength, comprising about 0.2 to about 0.8% carbon, about 0.5 to about 2.5% manganese, about 0.5 to about 1.5% chromium, about 0.25 to about 1.5% molybdenum, about 0.65 to about 4% copper, the remainder being substantially iron, the percent copper of the combined manganese and copper content ranging from about 20% to 80% as the carbon content ranges from about 0.2 to about 0.45% and from about 40% upwards as the carbon content ranges from about 0.45 to about 0.8%, tempered at a temperature below that at which copper precipitates when the carbon content is greater than about 0.45%, and substantially all said copper being retained in solid solution.

2. A deep hardened alloy steel article having good impact strength, comprising about 0.2 to about 0.8% carbon, about 0.5 to about 2.5% manganese, about 0.5 to about 1.5% chromium, about 0.25 to about 1.5% molybdenum, a minimum of 0.65% copper with a combined manganese and copper content of up to about 4%, the percent copper of the combined manganese and copper content in relation to the carbon content being as delineated between the lines A and B in Figure 2 of the drawing, the remainder being substantially iron, tempered at a temperature below that at which copper precipitates when the carbon content is greater than about 0.45%, and said copper being in solid solution.

3. An untempered alloy steel article hardened to a Rockwell C hardness of at least 40 through sections at least four inches thick having good toughness as indicated by impact tests and containing about 0.2 to 0.45% carbon, about 0.5 to 2.5% manganese, about 0.5 to 1.5% chromium, about 0.25 to 1.5% molybdenum, a minimum of 0.65% copper with a combined manganese and copper content of up to about 4%, the percent copper of the combined manganese and copper content being as delineated between the lines A and B in Figure 2 of the drawing for the corresponding carbon content, the remainder being substantially iron, said copper being in solid solution.

4. An alloy steel article hardened and tempered to a Rockwell C hardness of at least 59 through sections at least four inches thick, having good toughness as indicated by impact tests and containing about 0.45 to 0.8%

carbon, about 0.5 to 2.5% manganese, about 0.5 to 1.5% chromium, about 0.25 to 1.5% molybdenum, a minimum of 0.65% copper with a combined manganese and copper content of up to about 4%, the percent copper of the combined manganese and copper content being as delineated between the lines A and B in Figure 2 of the drawing for the corresponding carbon content, the remainder being substantially iron, tempered at a temperature below that at which copper precipitates, said copper being in solid solution.

5. A hardened alloy steel article having good toughness as indicated by impact tests and containing about 0.2 to 0.45% carbon, about 0.5 to 2.5% manganese, about 0.5 to 1.5% chromium, about 0.25 to 1.5% molybdenum, a minimum of 0.65% copper with a combined manganese and copper content of up to about 4%, and with the percent copper of the combined manganese and copper content ranging from about 20% to 80%, the remainder being substantially iron, said copper being retained in solid solution.

6. A hardened alloy steel article having good toughness as indicated by impact tests and containing about 0.45 to 0.8% carbon, about 0.5 to 2.5% manganese, about 0.5 to 1.5% chromium, about 0.25 to 1.5% molybdenum, a minimum of 0.65% copper with a combined manganese and copper content of up to about 4%, the percent copper of the combined manganese and copper content ranging from about 40 to 100% the remainder being substantially iron, tempered at a temperature below that at which copper precipitates, said copper being retained in solid solution.

7. A hardened alloy steel article having good toughness as indicated by impact tests at room temperature and at temperatures as low as -100° F. while being free of a transition temperature effect when cooled as low as -100° F., said article containing at least 0.1% carbon but less than 0.45%, about 0.5 to 2.5% manganese, about 0.5 to 1.5% chromium, about 0.25 to 1.5% molybdenum, a minimum of 0.65% copper with a combined manganese and copper content of up to about 4%, the percent copper of the combined manganese and copper content being as delineated between the lines A and B in Figure 2 of the drawing for the corresponding carbon content, the remainder being substantially iron, and said copper being retained in solid solution.

8. A deep hardened alloy steel article having good impact strength and hardened and tempered to a Rockwell C hardness of at least 59 through sections at least four inches thick, said article containing about 0.6 to about 0.8% carbon, about 0.5 to about 2.5% manganese, about 0.5 to about 1.5% chromium, about 0.25 to about 1.5% molybdenum, a minimum of 0.65% copper with a combined manganese and copper content of up to about 4%, the proportions of copper and manganese falling on or above the curve on the graph in Figure 1, the percent copper of the combined manganese and copper content being as delineated between the lines A and B in Figure 2 of the drawing for the corresponding carbon content, the remainder being substantially iron, tempered at a temperature below that at which copper precipitates, and said copper being retained in solid solution.

#### References Cited in the file of this patent

#### UNITED STATES PATENTS

- 2,104,979 Finkl \_\_\_\_\_ Jan. 11, 1938  
 2,104,980 Finkl \_\_\_\_\_ Jan. 11, 1938  
 2,336,247 Harris \_\_\_\_\_ Dec. 7, 1943

#### OTHER REFERENCES

Seabright: "The Selection and Hardening of Tool Steels," 1950, page 48. Published by McGraw-Hill Book Co., Inc., New York, N.Y.

"Electric Steel and Alloy Castings," brochure published by the Swedish Crucible Steel Co., Detroit, Mich. Date of first distribution was February 27, 1956.